

Aug. 20, 1963

H. EDER ETAL

3,101,277

METHOD OF RENDERING METALLIC SURFACES CORROSION RESISTANT

Filed April 27, 1959



INVENTORS  
HEINZ EDER  
BY SIEGFRIED BLOECK  
*Laurence R. Hobey*  
ATTORNEY

# United States Patent Office

3,101,277

Patented Aug. 20, 1963

1

3,101,277

## METHOD OF RENDERING METALLIC SURFACES CORROSION RESISTANT

Heinz Eder, Gauting, near Munich, and Siegfried Bloeck, Furth, Bavaria, Germany, assignors to Wacker-Chemie G.m.b.H., Munich, Bavaria, Germany

Filed Apr. 27, 1959, Ser. No. 803,899

Claims priority, application Germany Apr. 30, 1958  
9 Claims. (Cl. 117—132)

This invention relates to a method of imparting corrosion resistance to metallic surfaces by treating the surface with an organosilicon compound.

The flow diagram shown in the drawing illustrates the process of coating a metal surface with a monoorganosilicone material.

The problem of the corrosion of metal surfaces resulting from oxidation, acid attack and alkali attack of the surface has plagued producer and consumer alike. The use of protective coatings such as paints, lacquers, varnishes and the like has been a partial answer to this problem, but such materials are of limited effectiveness at high and low temperatures and against acid or alkali attack. Furthermore the mechanical integrity of such cured films is not satisfactory in that the film breaks under mechanical stresses such as bending, pulling and striking the metal and the cured films have not had satisfactory resistance to solvents and chemical agents in general.

In some cases, carefully produced oxide films are employed to protect aluminum, copper, magnesium and other metals from further corrosion. However the metallic surface must be substantially free of grease and other foreign matter or the metal must be pretreated prior to the surface oxidation to achieve a satisfactory degree of protection.

It is an object of this invention to introduce a simple, economical method of imparting corrosion resistance to metal surfaces. Another object is to produce acid resistant and alkali resistant sheets, foils and other forms of aluminum, copper, nickel and magnesium. Other objects and advantages are apparent or will be detailed in the disclosure and claims which follow.

This invention is a method of rendering metal surfaces corrosion resistant by coating the metal with a functional monoorganosilicon compound and thereafter heating the coated metal to a temperature below its melting point to cure the organosilicon composition.

The organosilicon compounds which are operable in this invention include silanes and siloxanes. The operable organosilicon compounds have an organic substituent to silicon ratio of from .9/1 to 1.2/1 and preferably about 1/1. The balance of the substituents attached to silicon in these compounds are selected from oxygen atoms, hydroxy radicals and alkoxy radicals. The operable silanes would be of the general formula



where each R is a monovalent hydrocarbon radical free of aliphatic unsaturation or halogenated monovalent hydrocarbon radical free of aliphatic unsaturation, each R' is hydrogen or alkyl, m has an average value of 0 to 1 inclusive, and n has an average value of .9 to 1.2 inclusive, preferably about 1.0. The organic radicals represented by R include alkyl radicals such as methyl, ethyl, butyl and octadecyl, aryl radicals such as phenyl and anthracyl, alkaryl radicals such as tolyl and methyl-naphthyl, aralkyl radicals such as benzyl and phenylethyl, and cycloaliphatic such as cyclohexyl and cyclobutyl. The preferred and most common silanes are methyl-, phenyl-, and ethyl-silanes.

The silanes can contain hydrogen substituents. There can be up to 1 hydrogen atom per silicon atom in such

2

silanes. In addition to the R substituents and the hydrogen atoms, functional substituents (OR') selected from hydroxy and alkoxy radicals are present on the silanes. Thus operable silanes include  $RSi(OH)_3$ ,  $RSi(OR')_3$ ,

5  $RSi(OH)(OR')_2$ ,  $RSi(OH)_2(OR')$ ,  $RHSi(OH)_2$   
 $RHSi(OH)(OR')$  and  $RHSi(OR')_2$

wherein each R' is an alkyl radical. Specific examples of operable silanes include methyltriethoxy silane, methyl-

10 tributoxy silane, methylmethoxy silane, methyltrihydroxy silane, methylhydroxydiethoxy silane, methyldihydroxy silane, phenyltrimethoxy silane, ethyltriethoxy silane, tolyldiethoxy silane, benzylhydroxy silane, and cyclo-

15 hexyltrimethoxy silane. It is apparent that R' can be the same or different in each operable silane. The silane employed can be a single specie or it can be mixtures of silanes. Limited amounts of diorganosilanes and  $SiO_2$  units can be tolerated in the mixture, but the closer the silane approximates an R/Si ratio of about 1, the better

20 the results achieved.

The organosilicon compounds employed can be siloxanes. The operable siloxanes are polymeric materials obtained by partial hydrolysis and condensation or by

25 complete hydrolysis and partial condensation or by partial hydrolysis and partial condensation of silanes. The silanes described above can be employed as starting materials in the production of the operable siloxanes. The silanes  $R_nH_mSi(OR')_{4-n-m}$  as defined above can be partially hydrolyzed by conventional techniques to produce

30 silanols such as  $R_nH_mSi(OR')_{4-n-m-x}(OH)_x$ . These silanols can then be condensed to siloxanes such as



Another method involved complete hydrolysis of the silane to produce siloxanes of the unit formula



40 followed by partial condensation to produce siloxanes of the unit formula  $R_nH_mSi(OH)_{4-n-m-x}O_{x/2}$ .

Another route to the operable siloxanes involves complete hydrolysis and partial condensation of chlorosilanes such as  $R_nH_mSiCl_{4-n-m}$  to produce the silanol



45 and the partial condensate  $R_nH_mSi(OH)_{4-n-m-x}O_{x/2}$ . Alcoholysis of the chlorosilanes produces alkoxy silanes from which the operable siloxanes can be prepared as noted above.

The organosilicon compounds employed are liquids soluble in organic solvents. They are usually relatively low molecular weight materials having viscosities of 1 to 10,000 cs. at 25° C. but they can be high viscosity materials of 1,000,000 cs. or more at 25° C.

50 The organosilicon compound is applied to the metal surface from a solvent solution, from an aqueous dispersion in an organic solvent, or from an emulsion. The solvent employed can be any organic solvent in which the particular organosilicon compound is soluble. Commonly employed as solvents are xylene, benzene, isopropyl, alcohol, acetic acid ethyl ester, Stoddard solvent, neutral minerals spirits, naphthas and other petroleum solvents, and so forth.

55 The metal is coated by any desired means. Such varied coating methods as brushing, spraying, dipping, flowing, and so forth are operable. It is desirable to form an unbroken film on the metal surface to secure even protection for the entire surface of the metal piece.

60 The metals can be in the form of sheets, bricks or pigs, foils or even completed parts such as gears, fenders for automobiles, flexible tubes for use as ducts, packing cases

and the like. While this invention is applicable to metals generally, it is of particular importance and usefulness with aluminum, nickel, copper, and magnesium as well as with alloys containing such metals.

The metal is coated as described above and is subsequently heated to a temperature of at least 350° C. but below the melting point of the metal. This heating step imparts a permanence and additional resistance to alkali and acid to the protective coating. It is often desirable to allow some or all of the solvent to evaporate from the coating film prior to heating. Thus the metal may be dipped in a tank containing a 10% solution of organosilicon compound in an organic solvent, removed and air-dried, then redipped if desired and again air-dried, then heated to above 350° C. The resultant coating is clear and hard. The coating can only be removed by extreme measures such as sandblasting or other abrasion means removing a surface layer from the metal itself.

The coated metal can be used without further treatment or it can be coated with lacquers, enamels, and so forth.

Aluminum tubes employed for packaging shaving cream were coated by dipping in a 10% by weight solution of methyltrimethoxy silane in xylene. The xylene was allowed to evaporate off the metal and the tubes were then heated to between 500° and 600° C. for above five minutes. The treated tubes were then filled with shaving cream having a pH of about 9.8. No reaction between shaving cream and tube could be discovered and the tube remained free of corrosion and deterioration after four months storage at 50° C.

A mustard-oil food product having a pH of 3.94 packed in tubes treated as above was stored for four months at 50° C. At the end of this storage period the tubes were opened. The mustard-oil product was unchanged in taste and remained completely usable as a foodstuff. The tubes were uncorroded and retained their original surface characteristics of brightness and smoothness.

A series of aluminum panels of 10 mils thickness were dipped in a 10 percent by weight solution of methyltrimethoxy silane in benzene. The panels were air-dried. The coated panels and some uncoated control panels were placed in an air circulating oven and heated to about 500° C. for 30 minutes. The coated panels and control panels were then immersed in concentrated hydrochloric acid for several hours. The coated panels showed substantially no attack at the end of the test but the un-treated control panels were gradually and progressively corroded and fell apart before the end of the test.

The foregoing are exemplary of the excellent results achieved through this invention. Similar results are achieved with copper, nickel and magnesium similarly coated. When phenyltrimethoxy silane, ethyldimethoxyhydroxy silane and methylhydrogenmethoxy siloxanes of the average unit formula  $CH_3H_aSi(OMe)_bO$ — where  $a$  has an average value of 0.25 and  $b$  has an average value of 0.75 are substituted for the silanes employed in the foregoing examples, similar corrosion resistance is imparted to the metals.

Corrosion resistance will be considerably increased when conventional catalysts are added which facilitate the hydrolysis of alkoxy silanes and accelerate the condensation of silicon organic compounds.

Substances facilitating hydrolysis include phosphoric acid and ferric chloride. Substances which accelerate condensation are all organometal compounds which in silicone chemistry are useful as condensation catalysts. Such substances include metal salts of carboxylic acids, alcoholates of heavy metals, metal chelates and the like, for example titanic acid esters, and organic zinc, tin, aluminum, lead, and zirconium compounds such as tetrabutyl titanate, dibutyl tin diacetate and dimaleinate, zirconium acetyl acetonate.

The aluminum surfaces are treated as described above.

The following experiments were conducted in order to test corrosion resistance:

Non-annealed collapsible aluminum tubes were treated with various silanes, mixtures of silanes, and the additives described above, and subsequently were annealed at 600° C. until they became soft. Then the tubes were filled with HCl which had been diluted with an equal amount of water. The periods which were necessary for 1 cm.<sup>3</sup>, 2 cm.<sup>3</sup>, or 3 cm.<sup>3</sup> of hydrogen to develop at room temperature were clocked. The results are tabulated below. The aluminum surface exposed to HCl was 17 cm.<sup>2</sup>.

Table

|                                                                                                      | Treatment of aluminum | Amount of H <sub>2</sub> , cm. <sup>3</sup> | Time   |
|------------------------------------------------------------------------------------------------------|-----------------------|---------------------------------------------|--------|
| (1) No treatment                                                                                     |                       | 1                                           | 1'30"  |
|                                                                                                      |                       | 2                                           | 1'45"  |
|                                                                                                      |                       | 3                                           | 1'54"  |
| (2) 10% $CH_3Si(OC_2H_5)_3$ in isopropyl alcohol                                                     |                       | 1                                           | 4'30"  |
|                                                                                                      |                       | 2                                           | 5'30"  |
|                                                                                                      |                       | 3                                           | 5'51"  |
| (3) 10% $(CH_3)_2Si(OC_2H_5)_2$ in isopropyl alcohol                                                 |                       | 1                                           | 2'20"  |
|                                                                                                      |                       | 2                                           | 2'40"  |
|                                                                                                      |                       | 3                                           | 2'50"  |
| (4) 10% $CH_3Si(OH)_3$ in isopropyl alcohol                                                          |                       | 1                                           | 10'47" |
|                                                                                                      |                       | 2                                           | 11'51" |
|                                                                                                      |                       | 3                                           | 12'32" |
| (5) 10% $CH_3Si(OC_2H_5)_3 + 3\%$ dibutyl tin dilaurate in isopropyl alcohol                         |                       | 1                                           | 6'30"  |
|                                                                                                      |                       | 2                                           | 7'19"  |
|                                                                                                      |                       | 3                                           | 7'50"  |
| (6) 10% $CH_3Si(OC_2H_5)_3 + 3\%$ zirconium acetyl acetate in isopropyl alcohol                      |                       | 1                                           | 7'49"  |
|                                                                                                      |                       | 2                                           | 8'23"  |
|                                                                                                      |                       | 3                                           | 8'47"  |
| (7) 10% $CH_3Si(OC_2H_5)_3 + 3\%$ phosphoric acid (89%) in isopropyl alcohol                         |                       | 1                                           | 10'05" |
|                                                                                                      |                       | 2                                           | 11'    |
|                                                                                                      |                       | 3                                           | 11'30" |
| (8) 6.6% $CH_3Si(OC_2H_5)_3 + 2.4\% (CH_3)_2Si(OC_2H_5)_2 + 1\%$ butyl titanate in isopropyl alcohol |                       | 1                                           | 15'07" |
|                                                                                                      |                       | 2                                           | 16'47" |
|                                                                                                      |                       | 3                                           | 17'37" |
| (9) 10% $CH_3Si(OH)_3 + 3\% H_3PO_4$ (89%)                                                           |                       | 1                                           | 19'    |
|                                                                                                      |                       | 2                                           | 20'    |
|                                                                                                      |                       | 3                                           | 20'40" |
| (10) 10% $(CH_3)_2Si(OC_2H_5)_2 + 3\%$ butyl titanate                                                |                       | 1                                           | 3'40"  |
|                                                                                                      |                       | 2                                           | 4'     |
|                                                                                                      |                       | 3                                           | 4'18"  |
| (11) 10% $CH_3Si(OH)_3 + 3\%$ butyl titanate                                                         |                       | 1                                           | 12'18" |
|                                                                                                      |                       | 2                                           | 13'55" |
|                                                                                                      |                       | 3                                           | 14'49" |

45

That which is claimed is:

1. The method of imparting corrosion resistance to metallic surfaces selected from the group consisting of aluminum, copper, nickel and magnesium consisting essentially of coating the surface of the metal with an organosilicon composition selected from the group consisting of at least one silane of the formula



55 and siloxanes of the unit formula



wherein each R is selected from the group consisting of monovalent hydrocarbon radicals free of aliphatic unsaturation and halogenated monovalent hydrocarbon radicals free of aliphatic unsaturation, each R' is selected from the group consisting of hydrogen atom and alkyl radicals, m has an average value of 0 to 1 inclusive, n has an average value of .9 to 1.2 inclusive and x has an average value of from 1 to 2 inclusive, the sum of  $n+m+x$  being less than 4, and thereafter heating the coated metal to a temperature of 350° C. to 600° C. until the organosilicon coating is cured.

2. The method of claim 1 wherein the organosilicon compound is applied to the metal surface from a solution in an organic solvent.

3. The method of claim 2 wherein aluminum is coated with a mixture of methyltrimethoxy silane and phenyltrimethoxy silane.

75

4. The method of claim 2 wherein the organosilicon compound is methyltrimethoxy silane.

5. The method of claim 2 wherein the organosilicon compound is methyltriethoxy silane.

6. The method of imparting corrosion resistance to metals selected from the group consisting of copper, nickel, aluminum, and magnesium, consisting essentially of coating the metal with at least one monoorganosilicon compound selected from the group consisting of silanes of the general formula  $R_nH_mSi(OR')_{4-n-m}$  wherein each R is selected from the group consisting of monovalent hydrocarbon radicals free of aliphatic unsaturation and halogenated monovalent hydrocarbon radicals free of aliphatic unsaturation, each R' is selected from the group consisting of the hydrogen atom and alkyl radicals,  $m$  has an average value of from 0 to 1 inclusive,  $n$  has an average value of from .9 to 1.2 inclusive, and partial hydrolyzates of such silanes, and heating the metal to the range above 350° C. and below the melting point of the metal until the organosilicon coating is cured.

7. The method of claim 6 wherein the organosilicon compound is applied to the metal surface from a solution in an organic solvent.

8. A method of imparting resistance to alkali and acid

to aluminum consisting essentially of coating the aluminum with a monoorganosilane of the formula



where each R is an alkyl radical, each R' is an alkyl radical and  $n$  has an average value of .9 to 1.2 inclusive and heating the coated metal to a temperature in the range 350° to 600° C. until the silane is cured.

9. The method of claim 8 wherein the organosilicon compound is applied to the metal surface from a solution in an organic solvent.

References Cited in the file of this patent

UNITED STATES PATENTS

|    |           |                 |               |
|----|-----------|-----------------|---------------|
| 15 | 2,258,218 | Rochow          | Oct. 7, 1941  |
|    | 2,386,466 | Hyde            | Oct. 9, 1945  |
|    | 2,643,964 | Smith-Johannsen | June 30, 1953 |
|    | 2,930,106 | Wrotnowski      | Mar. 29, 1960 |

20

FOREIGN PATENTS

|         |               |               |
|---------|---------------|---------------|
| 855,817 | Germany       | Nov. 17, 1952 |
| 563,995 | Great Britain | Sept. 8, 1944 |
| 650,131 | Great Britain | Feb. 14, 1951 |